

# United States Patent

[11] 3,609,438

[72] Inventors **Johannes Van Esdonk;  
Johannes Petrus Hornman, both of  
Emmasingel, Eindhoven, Netherlands**  
[21] Appl. No. **34,650**  
[22] Filed **May 5, 1970**  
[45] Patented **Sept. 28, 1971**  
[73] Assignee **U.S. Philips Corp.  
New York, N.Y.**  
[32] Priority **May 24, 1969**  
[33] **Netherlands**  
[31] **6908004**

[56] **References Cited**  
UNITED STATES PATENTS  
2,244,358 6/1941 Ewald..... 313/270 X  
2,386,790 10/1945 Gaun et al. .... 313/270 X  
2,393,057 1/1946 O'Larte et al. .... 313/85  
2,431,137 11/1947 O'Larte et al. .... 313/270 X  
2,468,136 4/1949 Taylor ..... 313/356  
2,611,676 9/1952 Pohle ..... 316/23  
*Primary Examiner—David Schonberg  
Assistant Examiner—Toby H. Kusmer  
Attorney—Frank R. Trifari*

[54] **ELECTRON GUN WITH NICKEL GRID PLATE  
AND COPPER-NICKEL ALLOY GRID CYLINDER**  
3 Claims, 3 Drawing Figs.

[52] **U.S. Cl.** ..... **313/311,  
313/270**  
[51] **Int. Cl.** ..... **H01j 1/14,  
H01j 1/48, H01j 19/06**  
[50] **Field of Search** ..... **313/270,  
311, 356**

**ABSTRACT:** An electron gun the first perforated electrode of which, which surrounds the cathode, consists of a perforated plate of nickel which is secured to a cylinder consisting of a copper-nickel alloy. (FIG. 3.)



PATENTED SEP 28 1971

3,609,438



Fig.1



Fig.2



Fig.3

INVENTORS  
JOHANNES VAN ESDONK  
JOHANNES P. HORNMAN  
BY

*Frank R. Jufair*  
AGENT

### ELECTRON GUN WITH NICKEL GRID PLATE AND COPPER-NICKEL ALLOY GRID CYLINDER

The invention relates to an electron gun consisting of a cathode opposite to which a metal plate is provided, which plate comprises one or several apertures for passing an electron current and is secured to a metal cylinder.

It is found that upon heating during the formation of the cathode, the perforated plate often warps at the area of the perforation so that the distance from the perforation to the cathode surface changes. This is a drawback in particular if the distance between the cathode and the plate is very small (approximately 100  $\mu$ ). In such electron guns the permitted deviation usually is approximately 10 percent, so  $\pm 5 \mu$ , as is described also in U.S. Pat. No. 2,611,676, column 1, line 13.

An electron gun is known from the U.S. Pat. No. 2,468,136 in which the deformation of the plate serving as a first grid is avoided in that the plate is soldered to a metallized surface of a graphite cylinder by means of nickel-, molybdenum- or platinum solder. However, the use of graphite is less desirable, since dust particles can be liberated thereby in the tube and the degassing will take a long time.

Furthermore it is known to provide a thin plate with a circumferential strengthening groove as is described in U.S. Pat. Nos. 2,393,057 and 2,611,676. It is found, however, that if the material of the plate has a thickness of less than 200  $\mu$ , said means in the known embodiments are no longer sufficient to prevent warping.

It has been found, however, that the deformation of such a plate can be avoided entirely if, according to the invention, the plate consists of nickel and the cylindrical part consists of a copper-nickel alloy. This alloy may contain from 40 to 75 percent by weight of nickel, but preferably an alloy is used of 55 percent by weight of copper and 45 percent by weight of nickel. The plate may be soldered to the cylinder, for example, by means of silver or be secured thereto by means of welding or diffusion. It has surprisingly been found that a nickel plate in a thickness of less than 200  $\mu$  remains entirely flat in the said combination of the materials.

In order that the invention may be readily carried into effect, it will now be described in greater detail, by way of example, with reference to the accompanying drawing, in which

FIG. 1 is a cross-sectional view of a known embodiment of an electron gun after the heating,

FIG. 2 is a cross-sectional view of a Wehnelt cylinder of another known construction, while

FIG. 3 is a cross-sectional view of a particular embodiment of an electron gun according to the invention.

Reference numeral 1 in FIG. 1 denotes the cathode support comprising the emitting layer 2 and a heater member 3. The 5 Wehnelt electrode consists of a perforated plate 4 which is secured to a supporting cylinder 5. The plate 4 and the cylinder 5 consist both of chromium-nickel steel.

It has been found that the originally flat plate 4, after heating during the decomposition and formation of the cathode 1, 10 2, is deformed as is shown in FIG. 1, so that the distance cathode-Wehnelt changes in spite of the presence of a circumferential groove 6.

The same is the case with the Wehnelt electrode 7 shown in FIG. 2 which consists entirely of chromium-nickel steel.

15 In FIG. 3 the perforated plate 9 consists of nickel, the supporting cylinder 8 of a copper-nickel alloy with 55 percent by weight of copper and 45 percent by weight of nickel. The plate 9 is soldered to the cylinder 8 by means of silver. The plate 9 also comprises a circumferential groove 6. The groove 6 is 20 preferably provided with the ridge facing the cathode side, since in that case the distance from the plate 9 to a following electrode can be smaller. It has been found that the plate 9 remains entirely flat. It has furthermore been found that this is not the case for other metal combinations for the plate 9 and the cylinder 8, respectively, for example, the combinations copper nickel-copper-nickel; chromium-nickel steel-copper nickel, copper-copper nickel; gold-copper nickel, and so on.

Although only one embodiment has been described the gun may also be formed differently without departing therefore from the scope of the present invention.

What is claimed is:

1. An electron gun comprising a cathode opposite to which is placed a metal plate having at least one aperture for passing an electron current, which plate comprises a circumferential strengthening groove and is secured to a metal cylinder, characterized in that the perforated plate consists of nickel having a thickness less than 200  $\mu$  and the cylinder consists of a suitable copper-nickel alloy.

2. An electron gun as claimed in claim 1, characterized in 35 that the copper-nickel alloy of the cylinder is from 40 to 75 percent by weight of nickel.

3. An electron gun as claimed in claim 1 characterized in 40 that the cylinder consists of an alloy of 55 percent by weight of copper and 45 percent by weight of nickel.